

## UNITED STATES PATENT OFFICE

1,939,378

PROCESS OF MAKING SAFETY PAPER BY  
ONE CONTINUOUS OPERATIONFrank S. Wood, Quincy, Mass., assignor to Inkset  
Safety Paper Co., a corporation of Massa-  
chussetsNo Drawing. Application November 8, 1930  
Serial No. 494,443

1 Claim. (Cl. 91—67.95)

My invention belongs to that class of safety papers in which the safety feature is imparted by treating ordinary writing paper with a chemical compound and more especially with the chemical compound for which an application for a patent was filed by me, on October 13, 1930, Serial Number 488,545.

This compound may be made in any quantity by dissolving one grain of tannic acid in each 10 gallon of water and adding 2½ to 5½ cubic centimeters of glacial acetic acid; to this add one-tenth of a gallon of decolorized iodine. Ordinary paper treated by my process is transmuted into safety paper which discolors and sets ink written on its surfaces when eradicators are used to remove the ink. If only 2 cubic centimeters of acetic acid are used the inkset will be thrown out and will not appear; the same thing will happen if 6 cubic centimeters or more of acetic 20 acid are used. Between 2½ and 5½ the different colors require different amounts to get the best results. Different grades of paper require special formulas to be worked out between the two extremes specified; but anyone skilled in the 25 art may quickly determine the best formula.

Heretofore, safety paper has required two or more operations or mechanical handlings. The first operation is the manufacture of the paper, to formula, in the usual way, leaving approximately 8% of moisture (water) in the paper. The second operation consists in some form of subsequent re-handling involving chemical treatment of the paper or printing or both which second operation costs, at least, as much as the 30 first; and this cost is considerably augmented if it be necessary to dry out any part of the water content left in the paper by the first operation.

The object of my invention is to eliminate the entire cost of the second operation and only 40 slightly increase the cost of the first by adapting it to better achieve the combined purposes of both in one continuous operation.

Paper has, in itself, an affinity for moisture called absorption that varies with its temperature, with the amount of moisture applied to it, and with the chemical character of the liquid supplying the moisture. When chemicals, for which paper has a strong affinity, are brought in contact with it, the natural tendency is to absorb 45 too much and become wet. In saturated paper, there is a moisture content of over 50%. After it has gone through three roll-pressings in the paper machine, it contains 40% of moisture. For the purposes of my invention, all paper is 50 wet which contains 9% or more of moisture,

and any degree of this range of wetness destroys the purpose of my process. It is, therefore, absolutely necessary to control the amount of moisture which the paper shall absorb to a very delicate degree. This is done by having the paper 60 in the right condition at a certain time, by having the right positive chemical for absorption by the negative paper, and by having the chemical applied to the paper under perfect mechanical and chemical control and regulation. All the essentials of perfect regulation, repressed affinity and mechanical and chemical supply, control and application are comprehended in the phrase, mechano-chemical absorption. Inherently, in order for the purpose of my process to be accomplished, the paper must be commercially dry 65 after the chemicals have been absorbed. No subsequent drying is essential; therefore there can be no previous wetness and especially no saturation; otherwise the paper would be spoiled. 70 It is a fact that my process is diametrically opposite to saturating, wringing, scraping, and then drying. Such methods all apply a surplus of moisture to the paper, too much moisture for my purpose, and then remove the surplus by 75 various methods of elimination subsequent to the application of moisture. With my process there is no wetting of the paper and no saturation. The paper is prevented from absorbing more than the amount of moisture to make it commercially dry by several mechanical and chemical balanced adjustments. A description of one of my experiments may illustrate and clear up anything lacking. I have taken a web of paper 80 dried out to a 3% moisture content as it came from the paper machine and have run that web, while still warm, through a machine comprised of a battery of spray-guns. These guns use compressed air at any desired pressure which spray a very fine fog of chemical upon the surfaces of 85 the paper, the liquid being sucked into the airblast before spraying. After being sprayed the paper was wound on a reel, still warm, and felt dry to the touch. It was found to contain 90 9% of moisture. This showed that it had absorbed 5% of chemical compound. It was neither saturated nor wet; it was dry and yet it had gone through no drying subsequent to the application of chemicals. The reason was that the moisture, being controlled and properly applied to the warm and super-dry paper, is absorbed by the paper without any perceptible moistening of its surface. By no possibility can any coating, saturating or oiling machine function in this 100 way when using other liquids than oil. Oil and 105 110

water work entirely different on paper. In my process, it is a combination of delicate means, conditions and balances, at just the right time and place that constitutes the novelty of my invention.

5 In brief, my invention consists of a process involving dehydration and subsequent mechanico-chemical absorption.

To this end, my invention eliminates the necessity of drying out the paper in a second handling, by dehydrating it as it is being made. This may be accomplished in two ways: Either by slowing down the speed of the paper-making machine and thus increase the time that the 10 paper is on the drying-rolls, or by adding two steam drying-rolls to the paper-making machine which gives the same result. This turns out a paper which is known to the art as "bone-dry".

In this condition, the bone-dry, hot paper is 15 threaded through the calender-stack for the purpose of giving it the desired finish which, in a writing paper, would probably be either a bond or a ledger finish. Having received its finish, the hot paper then is permitted to absorb approximately 8%, by weight, of a chemical compound adapted to transform the paper into safety paper. The chemical compound which supplies the moisture for absorption by the paper, may or may not be the chemical compound which 20 has hereinbefore been mentioned as the subject of separate patent proceedings, as my invention comprehends the use of any chemical compound which produces safety paper in one continuous operation through the two steps of dehydration and subsequent mechanico-chemical absorption.

The amount of moisture which any paper may absorb without damage is approximately 8% of its bone-dry weight; and this is also the approximate amount of chemical compound necessary 25 to produce a commercial, clear-stock safety paper by my process. While it is possible to strengthen and adapt a chemical formula to 1% or possibly 2% of water content left in the paper before being chemically treated, it is not safe to go beyond that, for the reason that any moisture left in the paper will, by so much, prevent the absorption of chemical compound, and insufficient chemical compound may have the same effect upon the paper as if it had never been treated or put through my process. Again, too much moisture, whether it be water, chemical compound or both will cause the paper to wind-up in a perfect honeycomb of wrinkles; an uneven 30 application of moisture will make the paper, draw, fold and even break, wasting both paper and compound. Hence, the necessity for a very fine adjustment of moisture in the form of chemical compound to be delivered to the paper for absorption. Having absorbed its predetermined, regulable and controlled quota of chemical compound, the paper then goes to the winder where it is made into a roll, thus completing the process of producing a safety paper at one continuous 35 operation.

60 There are several methods of applying the moisture of the chemical compound to the strong, attractive absorption given to the paper by dehydration, and it is essential that it shall be done through some form of moisture control. I have used squeeze-rolls with micrometer adjustment, also spraying nozzles under multiple valve controls; but I prefer that moistening-machine known to the paper trade as a brush-dampener, for the reason 70 that the amount of liquid delivered is regulable

to the fraction of 1%. However, any moisture-control device with a fine degree of adjustment will meet the demands of my process. Any attempt to apply the liquid to an upward traveling roll, such as a calender roll, and thence to the 80 paper, results in failure, for two reasons. First, from lack of moisture control; and second, from insufficient treatment. Such application floods the roll with liquid; the speed of the roll carries the compound upward until it contacts with the paper; but the speed of the paper together with the nip between the calender-rolls necessary to give the paper the desired finish, blocks absorption by the paper and results in partial treatment, only. Then again, this method of applying moisture is known in the art as a water-finish. Its effect is to give the paper a gloss. Since a gloss makes a bond finish impossible, only ledger paper may be turned out by such a method. Another objection to this method is that the calender-rolls wear unevenly. Where the surface 85 is not true, the worn part or parts act as a trough through which too much moisture will flow, causing the paper to pucker, fold and wind up in a damaged condition; while a little more wet will 90 cause the paper to break, wasting both paper and chemicals. It is to overcome such difficulties 95 that my process is designed.

Another serious obstacle that has many times 100 defeated the objects and purposes of their inventors was in having the chemical solution too powerful or off balance; that is to say, they were 105 too strong, too alkaline or too acid, any one of which will surely cause the paper to discolor after being chemically treated. This spoilage 110 and damage ends in complete fiasco. Besides 115 that, heavy damage was caused by ruining the brass rolls of the paper-making machine.

With my process, such outcomes are guarded 120 against by using a chemical compound so delicately balanced with effectual acids and bases as to be neutral in all of its contacts. It neither injures paper machines, equipment, paper nor 125 color. On the contrary, color is preserved by the chemical compound and the fiber of the paper 130 is improved and strengthened.

In many paper-mills, it is customary to set the calender-stack close to the drying-rolls. This makes it impracticable to set up an absorption unit between the steam-rolls and the calender. 135 If, however, there were sufficient space between the last drying-roll and the calender to install an absorption unit, there is no reason why the chemical compound could not be absorbed directly by the bone-dry paper which would, then, 140 be threaded through the calender where it would receive its finish and then go direct to the winder. Such a set-up would be consistent with the purposes of my invention and yet it might be impracticable to apply in most existing paper-mills, on account of lack of space to install the absorption unit at that point. Consequently, 145 for many installations, the absorption unit would preferably be set up between the calender-stack and the winder.

Hence, the second step in my process would 150 be an alternative step, i. e., it could either take place between the last drying-roll and the calender-stack or between the calender-stack and the winder. The result would be the same in either 155 case, a controlled absorption of chemical compound after dehydration, a condition consistent with any desired finish of the paper, and a commercial safety paper at one continuous operation.

I have found that the treatment of paper by my process strengthens the fiber so that paper of the same weight will register a higher bursting strength after going through my process than it did before. It is a fact that a pure sulphite paper made from wood pulp and put through my process has a higher bursting strength than an ordinary 60% rag paper.

It is a fact that paper of the most delicate and attractive tints may be made into a safety paper by my inventions without changing the shade of the tint, thus lending itself to the highest demands of the lithographer's art in colorful blends, contrasts and pictorial illustrations. This has heretofore been impossible with safety papers.

It is a fact that by giving a sulphite writing paper my process, its value, as represented by the wholesale selling price of inferior safety

papers, will be increased 3½ times; while the cost of production will be increased less than 10%.

What I claim as my invention and desire Letters Patent for is:

Steps in a process of making safety paper by one continuous operation comprising complete or approximate dehydration and subsequent controlled application and absorption of approximately 8% of water, decolorized iodine, tannic acid and acetic acid or their impregnating equivalents, adapted to transmute ordinary paper into a safety paper having the power of setting ink and causing discoloration when ink eradicator is applied to ink written on its surfaces, whereby said safety paper is produced commercially dry without requiring any further drying.

FRANK S. WOOD.

20

95

25

100

30

105

35

110

40

115

45

120

50

125

55

130

60

135

65

140

70

145

75

150

80

85

90

95